

March 21, 1961

T. W. PERKINS

2,976,201

COATED PANEL AND METHOD OF MAKING THE SAME

Filed Dec. 29, 1958

FIG. 1



FIG. 2



FIG. 3



INVENTOR.  
THEROLD W. PERKINS  
BY *T. W. Dysart*  
HIS ATTORNEY

1

2,976,201

## COATED PANEL AND METHOD OF MAKING THE SAME

Therold W. Perkins, Fern Creek, Ky., assignor to General Electric Company, a corporation of New York

Filed Dec. 29, 1958, Ser. No. 783,430

2 Claims. (Cl. 154—116)

This invention relates to sheet metal panels provided with a plastic coating, and has as its general object the provision of an improved panel of this type and an effective method of making such panels.

Further objects and advantages of the invention will become apparent as the following description proceeds, and the features of novelty which characterize the invention will be pointed out with particularity in the claims annexed to and forming a part of this specification.

Briefly stated, in accordance with one aspect of my invention there is provided a method of making coated sheet metal panels which includes the steps of placing a protective strip of formed plastic material on the edge of the panel (which in the past has proved to be difficult to coat effectively with a coating deposited in liquid form), depositing a layer of plastic material on the surface of the panel in lapped relation with the protective strip, and curing the plastic material so as to provide a panel having a continuous uninterrupted film bonded to both the panel surface and the edge of the panel.

For a better understanding of this invention reference may be made to the following description and the accompanying drawing in which:

Fig. 1 is a fragmentary perspective view, in section, of the edge portion of a sheet metal panel to which this invention is applicable.

Fig. 2 is similar to Fig. 1 but shows the panel in an intermediate stage of the coating method disclosed herein.

Fig. 3 is similar to Fig. 1 but shows the panel of the present invention in its completed form.

The present invention has been found to be particularly useful in the manufacture of tubs for dishwashing machines, and in the drawing the three figures show the top edge portion of a dishwasher tub the sides and bottoms of which are formed of sheet steel with the top edges thereof having the flanged construction illustrated so as to provide a seat for a tub cover. However, it will be understood that this particular embodiment of the invention has been shown for illustrative purposes only, and that the invention is applicable to the coating of sheet metal panels of various shapes and sizes in which it is necessary to protect an edge portion of the panel against corrosion and the like.

Referring to the drawing, the numeral 1 designates a sheet metal panel forming one of the side walls of a dishwasher tub, the top edge of the panel having a reverse bend portion 2 arranged to provide a seat 3 for a tub cover (not shown). An edge portion 4 of the panel is bent upwardly from seat portion 3, the edge 5 of edge portion 4 being the uppermost part of panel 1.

While the outer surface 6 of panel 1 is not subject to severe corrosion, the inner surface 7, being one of the inner surfaces of the dishwasher tub, must be protected against the corrosive effects of detergents, food acids and the like. Accordingly, coatings of a thermoplastic plastic material, such as plastisol, have been used in the past to coat the entire inner surface of the dishwasher tub, and

2

since upper edge 5 of the panel is frequently exposed to some of the fluid circulated within the dishwasher attempts have been made to thoroughly coat this edge surface as well. While plastisol in liquid form may be successfully and effectively sprayed on flat surfaces such as inner surface 7, the spray coating of edge portions of the panel has not proved to be completely effective, it being difficult to make sure that a coating of proper thickness over the entire edge is always achieved. As a practical matter, thin spots and gaps in the plastisol coating on edge 5 sometime develop and the corrosive action which begins in such areas may proceed into the panel along the surface and under the plastisol coating thereon. Such corrosion may proceed to the point where adhesion of the plastisol coating is destroyed, thus permitting the coating to loosen and eventually expose the inner surface of the sheet metal.

In accordance with the present invention I provide a protective strip formed of a suitable plastic material and shaped so as to completely cover edge 5 of panel 1, making it unnecessary to attempt to spray coat this portion of the panel. After the protective strip has been placed on the edge of the panel a layer of plastic material is deposited on the inner surface of the panel in liquid form, by spraying or other suitable means. The plastic material is also deposited on the adjacent portion of the protective strip overlying the same surface so as to form a continuous film. The entire coated panel may then be cured, by heat or other suitable means depending upon the particular plastic material used, so as to bond the protective strip to the edge portion of the panel and also to bond the coating applied in liquid form to the surface of the panel and to the adjacent portion of the protective strip in the area in which these two coatings overlap. As shown in Fig. 3, the resulting product is provided with a protective coating, which may be of any desired thickness, on all surfaces and edges requiring corrosion protection.

Having generally described the method and product of my invention, one particular example will now be described. After the sheet metal panel illustrated in the drawing has been formed into the configuration shown therein and described above, the panel is thoroughly cleaned by subjecting it to an alkali cleaning process followed by a zinc phosphate coating. After these cleaning steps, the edge portion 4 of the panel is coated with a phenolic base primer adhesive or any other suitable primer adhesive. Next, a thin coating of low viscosity plastisol is applied to edge portion 4 to obtain good adhesion, and then a protective strip 8 of U-shaped configuration and formed of a high resin content vinyl plastic material is placed on the edge portion of the panel, as shown in Fig. 2. Preferably, protective strip 8 is then partially heat cured by subjecting the panel to a temperature of 290° F. for a period of approximately 20 minutes. The inner surface 7 of panel 1 is then spray coated with plastisol, care being taken to extend the coating 9 up over the adjacent portion of the protective strip as shown in Fig. 3. Finally, the panel is again heat cured at 400° F. for approximately 20 minutes so as to complete the curing of both the protective strip 8 and the inner sprayed-on coating 9. Upon completion of this process, panel 1 is provided with a protective plastic coating which completely covers the edges of the panel as well as the flat surfaces thereof.

While I have shown and described a particular embodiment of my invention, I do not desire the invention to be limited to the particular construction and order of the method steps disclosed, and I intend by the appended claims to cover all modifications within the true spirit and scope of my invention.

## What I claim:

1. A method of coating a sheet metal panel with a thermoplastic material comprising the steps of cleaning the panel, applying a primer coat to the metal, securing a U-shaped protective strip of formed thermoplastic material on the edge of the panel, spraying a layer of thermoplastic material in liquid form on the surface of the panel and on the adjacent portion of said protective strip overlying said surface, and finally heating said panel so as to cure said thermoplastic material and bond said protective strip to said panel, said thermoplastic material being thereby bonded to said panel and fused to the protective strip so as to form a continuous corrosion resistant coating on the surface and edge portions of the panel. 10
2. The method of coating a sheet metal panel with a thermoplastic material comprising the steps of cleaning the panel, applying a primer coat to the panel, coating 15

one side and the edge of the panel with a thermoplastic material by spraying a layer of thermoplastic material in liquid form on the surface of the panel and securing a U-shaped protective strip of formed thermoplastic material around the edge of the panel, there being a lap joint between the sprayed layer and the protective strip, and finally heating said panel so as to cure the thermoplastic materials and bond said protective strip to said panel, said thermoplastic layer being thereby bonded to said panel and fused to the protective strip so as to form a continuous corrosion resistant coating on the surface and edge portion of the panel. 4

## References Cited in the file of this patent

## UNITED STATES PATENTS

2,696,865 Seiler ----- Dec. 14, 1954